



US009956615B2

(12) **United States Patent**  
**Hanusiak et al.**

(10) **Patent No.:** **US 9,956,615 B2**  
(45) **Date of Patent:** **May 1, 2018**

(54) **TITANIUM POWDER PRODUCTION APPARATUS AND METHOD**

(75) Inventors: **William M. Hanusiak**, Windermere, FL (US); **Dale R. McBride**, Bruceton Mills, WV (US)

(73) Assignee: **CARPENTER TECHNOLOGY CORPORATION**, Philadelphia, PA (US)

(\*) Notice: Subject to any disclaimer, the term of this patent is extended or adjusted under 35 U.S.C. 154(b) by 457 days.

(21) Appl. No.: **13/414,769**

(22) Filed: **Mar. 8, 2012**

(65) **Prior Publication Data**

US 2013/0233129 A1 Sep. 12, 2013

(51) **Int. Cl.**

*B22F 9/08* (2006.01)  
*C22B 34/12* (2006.01)

(52) **U.S. Cl.**

CPC ..... *B22F 9/082* (2013.01); *B22F 2009/0888* (2013.01); *B22F 2009/0892* (2013.01); *B22F 2999/00* (2013.01)

(58) **Field of Classification Search**

None

See application file for complete search history.

(56) **References Cited**

U.S. PATENT DOCUMENTS

|               |         |                            |
|---------------|---------|----------------------------|
| 2,874,953 A   | 2/1959  | Rogers et al.              |
| 3,734,480 A   | 5/1973  | Zanis et al.               |
| 4,188,368 A * | 2/1980  | Frosch et al. .... 423/350 |
| 4,544,404 A * | 10/1985 | Yolton et al. .... 75/338  |
| 4,654,858 A   | 3/1987  | Rowe                       |
| 5,164,097 A * | 11/1992 | Wang et al. .... 222/590   |
| 5,198,017 A * | 3/1993  | Mourer et al. .... 75/345  |
| 5,213,610 A   | 5/1993  | Yolton et al.              |
| 5,707,419 A   | 1/1998  | Tsantrizos et al.          |

\* cited by examiner

*Primary Examiner* — George Wyszomierski

(74) *Attorney, Agent, or Firm* — Nixon & Vanderhye, P.C.

(57) **ABSTRACT**

A method and apparatus for producing titanium metal powder from a melt. The apparatus includes an atomization chamber having an inner wall that is coated with or formed entirely of CP-Ti to prevent contamination of titanium metal powder therein. The inner surfaces of all components of the apparatus in a flow path following the atomization chamber may also be coated with or formed entirely of CP-Ti.

**5 Claims, 1 Drawing Sheet**





## 1

TITANIUM POWDER PRODUCTION  
APPARATUS AND METHOD

## BACKGROUND OF THE INVENTION

## 1. Field of the Invention

The present invention relates to a titanium powder production apparatus and method and, more particularly, to such an apparatus and method that prevents contamination of the titanium powder.

## 2. Description of the Background Art

Powder metallurgy is an important technology in the production of parts made out of titanium for critical applications such as aerospace. Titanium metal powder is the basic raw material in this process path. Atomization using an inert gas such as argon is a commonly used process to produce uniform spherical-shaped powders that possess high packing densities. A typical device for gas atomization consists of a liquid metal stream supply source, the atomizing gas jet, and a cooling chamber. The free-falling stream of molten titanium is impinged with inert gas jet at a high velocity, the atomized droplets of titanium solidify in flight through the chamber, and are collected at the bottom of the chamber. Extremely high values of cooling rates during the solidification of the droplets are desired in order to obtain very specific, controlled structures. Several aspects of design and construction of the atomization chamber are important:

1. The chamber must be constructed with a material that does not react with titanium up on contact;
2. The chamber must be large enough to allow titanium droplets to solidify before they come in contact with the walls or bottom section of the chamber;
3. The chamber should allow complete evacuation to prevent atmospheric contamination; and
4. The chamber design should allow easy access for complete cleaning and inspection of its interior.

Stainless steel is the most commonly used material for the construction of titanium atomization chambers. There exists a possibility that some of titanium droplets hit the atomization chamber before solidification. These droplets react with stainless steel producing low-melting point compounds that are brittle in nature. These compounds enter into the titanium powder stream as contaminants and remain undetected in standard quality control techniques. Components made out of these contaminated powders experience catastrophic in-service failures.

## BRIEF SUMMARY OF THE INVENTION

In accordance with the present invention, the powder metal contamination can be eliminated by lining the metal powder flow path or fabricating the metal powder flow path beyond the atomization stage with a metal that is non-contaminating to the metal powder being produced.

In the case of titanium metal powder, the wall of the atomization chamber preferably is lined or fabricated from CP-Ti, a commercially pure titanium. Although a titanium alloy such as Ti-6Al-4V could be used for the liner or chamber wall if the titanium powder metal being produced is Ti-6Al-4V, CP-Ti is universally acceptable with any titanium alloy since all titanium alloys are primarily composed of titanium metal.

This solution applies to any powder metal production system, since metal contamination can be created in the chamber cleaning operation, it is particularly applicable to metal powder production from a melt as this method experiences occasional powder ball to chamber wall bonding.

## 2

Atomization from a melt includes gas atomization (GA) in which a molten stream of metal is impinged by a high velocity inert gas jet to form a powder, and spinning electrode methods (PREP) in which the end of a metal bar is melted while the bar rotates rapidly throwing off metal droplets.

In either case, melting can be achieved by electron beam, plasma torch, electrical arc, induction heating, laser heating or any other sufficiently powerful heating method.

## BRIEF DESCRIPTION OF THE DRAWING

FIG. 1 is a schematic view of a portion of apparatus for producing titanium powder.

## DETAILED DESCRIPTION OF THE INVENTION

Referring to FIG. 1, apparatus 10 for producing titanium powder includes an atomization or hot spray chamber 12 for receiving an atomized liquid metal stream supply from a known system such as a cold wall induction guiding system, an electrode induction melting gas atomization process, a plasma-melting induction-guiding gas atomization method, a triple melt process or any other known system. The powder from the atomization chamber 12 is passed through a conveying tube 14, through a cyclone separator 16 and then into powder containers 18, as shown in FIG. 1.

In accordance with the present invention, the entire inside surface 20 of the atomization chamber 12 is coated with or formed of CP-Ti to prevent contamination of titanium metal powder being produced from a melt including titanium powder metal as hereinbefore described. As an illustrative example, a coating of CP-Ti on the inner surface 20 of the atomization chamber 12 may have a thickness of about 2 mm. The atomization chamber may be formed of any suitable material, such as stainless steel. Alternatively, the atomization chamber 12 can be formed of CP-Ti instead of a coating of CP-Ti on the inner surface formed of another material.

To further ensure against contamination of the titanium powder, the entire flow path after the atomization chamber 12 may be coated with or formed of CP-Ti. For example, the conveying tube 14, cyclone separator 16 and powder containers 18 may all be formed of or coated internally with CP-Ti to prevent any contamination of the titanium powder.

Although a titanium alloy such as Ti-6Al-4V could be used for the liner or chamber wall 20 in the atomization chamber 12 and subsequent flow path if the titanium powder metal being processed is Ti-6Al-4V, CP-Ti is universally acceptable in any titanium alloy since all titanium alloys are primarily composed of titanium metal.

While the invention has been described in connection with what is presently considered to be the most practical and preferred embodiments, it is to be understood that the invention is not to be limited to the disclosed embodiments, but on the contrary, is intended to cover various modifications and equivalent arrangements included within the spirit and scope of the appended claims.

The invention claimed is:

1. Apparatus for producing titanium metal powder from a melt including titanium powder metal, comprising an atomization chamber having an inner wall that is coated with or formed entirely of commercially pure titanium to prevent contamination of titanium metal powder therein, further comprising a powder conveying tube connected to an exit opening of the atomization chamber, a cyclone separator

connected to the powder conveying tube and a powder container connected to the cyclone separator, and wherein inner surfaces of the conveying tube, the cyclone separator and the powder container are coated with or formed entirely of commercially pure titanium.

2. A method for preventing contamination of titanium powder in an apparatus for producing it from a melt including titanium powder metal, the apparatus having an atomization chamber with an inner wall, comprising coating the inner wall or forming it entirely of commercially pure titanium, wherein the apparatus further comprises a conveying tube, a cyclone separator and a powder container in a flow path following the atomization chamber, and coating inner surfaces of the conveying tube, the cyclone separator and the powder container with commercially pure titanium or forming the inner surfaces thereof entirely of commercially pure titanium.

3. A method for preventing contamination of titanium powder in an apparatus for producing it from a melt including titanium powder metal, the apparatus having an atomi-

zation chamber with an inner wall, comprising coating the inner wall or forming it entirely of commercially pure titanium, and further comprising coating inner surfaces of all components of the apparatus in a flow path following the atomization chamber with commercially pure titanium or forming the inner surfaces entirely of commercially pure titanium.

4. Apparatus for producing titanium metal powder from a melt including titanium powder metal, comprising an atomization chamber having an inner wall that is coated with commercially pure titanium to prevent contamination of titanium metal powder therein, wherein the inner wall is formed of stainless steel.

5. A method for preventing contamination of titanium powder in an apparatus for producing it from a melt including titanium powder metal, the apparatus having an atomization chamber with an inner wall, comprising coating the inner wall with commercially pure titanium, wherein the inner wall is formed of stainless steel.

\* \* \* \* \*